

## UNITED STATES PATENT OFFICE

1,972,693

FORMATION OF DENSE, HIGHLY LUSTROUS  
AND IMPERVIOUS DEPOSITS OF NICKEL

Max Schlötter, Berlin, Germany

No Drawing. Application November 10, 1932,  
Serial No. 642,022

15 Claims. (Cl. 204—14)

My invention relates to the formation of dense, highly lustrous and impervious deposits of nickel and similar metals and to a process of electrodeposition of such deposits.

5 When nickel is deposited electrolytically from a solution of the salts heretofore used for nickel plating, a dull deposit is obtained which must be subsequently polished mechanically to obtain a glossy or lustrous surface. By the use of colloids 10 of high molecular weight (about 5000 or more) in the plating baths heretofore employed, it has been possible to obtain a deposit of high lustre but the mechanical properties of the deposits thus obtained are adversely affected. The resistance 15 of such deposits against corrosion, cracking and peeling are reduced by the action of the colloids and the deposits are brittle and not suitable for further working.

An object of the present invention is to provide 20 a deposit or coating of nickel that has an inherent high gloss, high resistance to abrasion and to penetration and corrosion.

A further object is to provide a process by which 25 a nickel deposit with a high gloss may be formed electrolytically.

In my invention, I form a deposit in which the size of the crystals is much smaller than in any deposits heretofore obtainable and, therefore, one in which the surface formed by the crystals is so 30 fine grained as to produce, without mechanical polishing, an appearance of high lustre. The deposition of the metal in crystals of extreme fineness also gives a hard, compact deposit that is 35 highly resistant to scratching, abrasion or corrosion. This glossy nickel deposit may be produced in any desired thickness up to one millimeter and over.

I accomplish the above deposits by electrolytic 40 deposition in the presence of organic colloids of much smaller molecular weights than those of colloids heretofore used, that is, of a molecular weight less than 5000. In the electrodeposition of the metal these colloids are deposited into the deposit by kataphoresis, adsorption or other capillary action. Heretofore, when heavy or high 45 molecular weight colloids have been used, their size disturbed or interfered with the union of the crystals, whereas, with colloidal material of smaller molecular weight, less space is taken by the colloid and the interlacing or union of the crystals is not impaired, and adherent, fine grained or high gloss deposits may be obtained of a thickness up to a millimeter or over.

The material to be suitable for this purpose 50 must dissolve in water to form a colloidal solu-

tion and be capable of being deposited by adsorption or kataphoresis in small quantities to delay the speed of growth of the crystals. The growth of the crystal is thereby retarded and smaller crystals are obtained.

The following are examples of electrolytic baths for the deposition of nickel by my invention:

## Example I

|                           | Grams |
|---------------------------|-------|
| Nickel sulphate           | 160   |
| Nickel benzoldisulphonate | 30    |
| Boric acid                | 30    |

in sufficient water to give a pH value of 2.5 to 4.5.

## Example II

|                                 | Grams |
|---------------------------------|-------|
| Nickel chloride                 | 160   |
| Nickel naphthalenetrisulphonate | 30    |
| Boric acid                      | 30    |

and water sufficient to give a pH value of 2.5 to 4.5.

It will be understood that other nickel salts may be used as electrolytes and that other aromatic poly-sulphonates may be employed and the proper acidity may be obtained by other acids than boric acid.

Deposits of nickel made by the use of the above baths have very small crystals, as small as about one ten-thousandth of a millimeter, and even less, as determined by a magnified X-ray photograph. The size of these crystals is so small that the surface of the deposit has the appearance of a high polish or lustre. The nickel plated surface may be used without polishing either as a finish coat or as a base for a deposit of chromium or other metal. Avoidance of the necessity for polishing avoids the attendant danger of removing the coating or thinning it excessively.

The action of the colloids is, in a sense, mechanical in interfering with the building up of larger crystals due to the electrodeposition by kataphoresis on the deposit and thus breaking the continuity of the crystals. It will be understood, therefore, that the above examples are illustrative rather than as limiting, and that other colloids than those mentioned may be used.

What I claim is:

1. A high gloss compact and adherent deposit

110

- of nickel having a crystal size of less than about one ten-thousandth of a millimeter.
2. A high gloss compact and adherent deposit of nickel having a crystal size of less than about one ten-thousandth of a millimeter and containing a small amount of a colloidal organic nickel salt.
3. A metal base having a surface deposit of nickel, the crystal size in said deposit being less than one ten-thousandth of a millimeter.
4. A process for the electrodeposition of nickel which comprises passing electric current from an anode to a cathode through an electrolyte bath of nickel in the presence in said bath of nickel benzenedisulphonate.
5. A process for the electrodeposition of nickel which comprises passing electric current from an anode to a cathode through an electrolyte bath of nickel in the presence in said bath of nickel naphthalenetrisulphonate.
6. A process for the electrodeposition of nickel having a crystal size less than 1/10000th of a millimeter which comprises passing electric current from an anode to a cathode through an electrolyte bath in the presence of an aromatic sulphonate containing more than one sulphonate acid group.
7. A process for the electrodeposition of nickel having a crystal size less than 1/10000th of a millimeter which comprises passing electric current from an anode to a cathode through an electrolyte bath of nickel in the presence in said bath of an aromatic poly-sulphonate of nickel.
8. A high gloss compact and adherent deposit of nickel having a crystal size of less than about 1/10000th of a millimeter and a thickness substantially greater than 1/10000th of a millimeter.
9. A process for the electrodeposition of nickel which comprises passing an electric current from an anode to a cathode through an electrolytic bath of nickel in the presence in said bath of a benzene sulphonate containing more than one and less than four sulphonate acid groups.

10. A process for the electrodeposition of nickel which comprises passing electric current from an anode to a cathode through an electrolyte bath of nickel in the presence in said bath of naphthalene sulphonate containing more than one and less than four sulphonate acid groups.

11. A process for the electrodeposition of nickel which comprises passing electric current from an anode to a cathode through an electrolyte bath in the presence of an aromatic sulphonate containing more than one and less than four sulphonate acid groups and containing a chloride.

12. A process for the electrodeposition of nickel which comprises passing electric current from an anode to a cathode through an electrolyte bath in the presence in said bath of a nickel aromatic poly-sulphonate of less than four sulphonate acid groups and containing a chloride.

13. A process for the electrodeposition of nickel which comprises passing electric current from an anode to a cathode through an electrolyte bath in the presence in said bath of a nickel aromatic poly-sulphonate of less than four sulphonate acid groups.

14. A process for the electrodeposition of nickel having a crystal size less than 1/10000th of a millimeter which comprises passing electric current from an anode to a cathode through an electrolyte bath having a pH value of between about 2.5 to 4.5 in the presence of an aromatic sulphonate containing more than one sulphonate acid group.

15. A process for the electrodeposition of nickel having a crystal size less than 1/10000th of a millimeter which comprises passing electric current from an anode to a cathode through an electrolyte bath of nickel having a pH value of between 2.5 and 4.5 in the presence in said bath of an aromatic poly-sulphonate of nickel.

MAX SCHLÖTTER. 115

45 120

50 125

55 130

60 135

65 140

70 145

75 150